

May 11, 1971

A. F. ARMINGTON ET AL

3,578,414

APPARATUS FOR GROWTH OF LARGE CRYSTALS IN GELS

Filed Oct. 24, 1967



FIG. 1



FIG. 2



FIG. 4



FIG. 3



FIG 5

INVENTORS  
ALTON F. ARMINGTON,  
JOHN J. O'CONNOR  
BY Harry P. Herbert Jr  
William J. O'Brien  
ATTORNEYS

1

3,578,414

## APPARATUS FOR GROWTH OF LARGE CRYSTALS IN GELS

Alton F. Armington, Lexington, and John J. O'Connor, Arlington, Mass., assignors to the United States of America as represented by the Secretary of the Air Force

Filed Oct. 24, 1967, Ser. No. 677,791  
Int. Cl. B01d 9/02

U.S. Cl. 23—273

3 Claims

### ABSTRACT OF THE DISCLOSURE

An apparatus for growing single crystals of a relatively large size having first and second reactant containing reservoirs respectively possessing relatively large volumes in relation to the volume of a crystal growing chamber positioned in a horizontal relationship between the reservoirs and interconnected thereto. Crystal growth is effected in a gel matrix positioned within the crystal growing chamber with the first and second reservoirs containing the required crystal growing solutions needed to bring about crystal growth.

### BACKGROUND OF THE INVENTION

This invention relates to an apparatus for growing electromagnetic crystals at room temperature. More particularly, this invention concerns itself with an apparatus for growing large single crystals within a gel matrix which comprises large reactant material storage reservoirs positioned on both sides of and interconnected to a crystal growing chamber containing the gel matrix.

The increased use of single crystals in a variety of electronic applications has created a need for the development of crystalline materials that possess an overall high quality and the requisite electromagnetic characteristics. In general, crystal growing techniques involve the use of elevated temperatures and high vacuums. One system often employed to effect the growth of crystalline materials such as cuprous chloride, cuprous bromide, silver chloride, lead sulfide and other well-known electromagnetic crystals is the melt method which utilizes extremely high temperatures. The use of high temperatures, however, often produces defective crystals. The presence of a phase transition below the melting point of the material often produces stress and strain faults within the crystal structure. The stress and strain faults are also further intensified by various temperature gradients during the period of cooling to room temperature. Contamination from container materials also constitutes another serious disadvantage when using the melt method to effect crystalline growth.

To overcome the problems and disadvantages inherent with the use of elevated temperature conditions, it has been found that single crystals can be grown within a gel matrix. The method, in general, involves the generation of a chemical reaction within the gel matrix between two soluble reactant materials to form an insoluble reaction product. The placing of a chemically complexed crystalline containing solution in contact with a gel matrix is another method which has proved to be feasible for producing high quality single crystals. The chemical complexing agent diffuses through the gel at a faster rate than the desired crystalline containing material. The crystalline containing material is rendered insoluble by dilution and precipitates out as single crystals. Although this latter method of using complexing agents has proved effective in growing high quality crystals, it has not produced crystals of a size large enough for use in certain applications.

2

The lack of uniform concentration gradients and the problem of maintaining stationary concentration gradients within the gel matrix appears to be responsible for the growth of the relatively small size crystals obtained heretofore.

### SUMMARY OF THE INVENTION

In accordance with the present invention, it has been found that relatively large single crystals, free of defects and of an overall high quality can be formed within a gel matrix by utilizing an apparatus comprising a first and second reactant containing reservoir means which possess a large volume area. The reservoir means are positioned on each side of a crystal growing chamber and are interconnected therewith. The volumetric ratio between the individual reservoirs and the crystal growing chamber is at least greater than 10 to 1. The large volumetric ratio is needed to prevent the creation of non-uniform concentration gradients within the gel matrix contained in the chamber.

The apparatus of the invention provides a simple and economical means for growing large single crystals of a uniform diameter at room temperatures and ambient pressures without resorting to the complex control problems encountered in high temperature crystal growing methods.

Accordingly, the primary object of this invention is to provide an apparatus for growing large single crystals at room temperature.

Another object of this invention is to provide an apparatus for growing electromagnetic crystals within a gel matrix.

Still another object of this invention is to provide an apparatus that is particularly adapted for controlling the concentration gradients of crystal growing solutions within a gel matrix.

A further object of this invention is to provide an apparatus for growing single crystals within a gel matrix that allows a uniform and stationary concentration gradient to be set up in the gel matrix.

Still a further object of this invention is to provide an apparatus which allows for the growth of electromagnetic single crystals of large size in a simple and economical manner.

The above and still further objects, advantages and features of this invention will become apparent upon consideration of the following detailed description thereof taken in conjunction with the accompanying drawings.

### BRIEF DESCRIPTION OF THE DRAWINGS

In the drawings, the figures represent illustrative embodiments of the invention:

FIG. 1 is a front elevational view of one embodiment of the invention illustrating its various elements.

FIGS. 2, 3 and 4 are front elevational views of additional embodiments of the apparatus of this invention; and

FIG. 5 is an enlarged front elevational view of a portion of the apparatus disclosed in FIG. 1.

In all the figures, like elements are represented by like numerals.

### DESCRIPTION OF THE PREFERRED EMBODIMENTS

Referring to FIG. 1, there is shown a first reservoir 10 for supplying a reactant material to a crystal growing chamber 12. A second reservoir 14 is positioned in a horizontal relationship to the chamber 12 in the same manner as reservoir 10. Reservoirs 10 and 14 are interconnected respectively to chamber 12 by means of conduits 16, 18, 20 and 22. The crystal growing chamber 12 is in the convenient form of a U-tube and contains a gel matrix 24.

The large reservoirs 10 and 14 are positioned on both sides of the chamber 12 in a horizontal relationship rather than in a vertical relationship over the gel in order to minimize pressure on the gel 24, particularly when filling the reservoirs with crystal growing solutions. A volumetric ratio between the individual volumes of reservoirs 10 and 14 and the volume of the crystal growing chamber of greater than 10 to 1 is necessary in order to effectuate crystal growth. Volumetric ratios in the range of about 15 to 1 are preferred. Larger ratios may be employed, but do not contribute to the effectiveness of crystal growth. The use of the large reservoirs allows a uniform concentration gradient to be set up and maintained in a stationary manner within the gel matrix 24 of the chamber 12. Thus, since the crystals form at specific concentrations and the concentration gradient is stationary in this apparatus, large crystals can be formed at the location where the proper concentration is present.

The apparatus of FIG. 1 has been successfully employed for the formation of cuprous chloride crystals within a gel matrix by the dilution of a saturated cuprous chloride solution complexed in hydrochloric acid. The following detailed example is presented to illustrate the operation of the apparatus disclosed herein.

#### Example

A silica gel 24 is first prepared by titrating 1 N hydrochloric acid with 0.5 molar sodium metasilicate to a pH of about 5. The gel 24 is poured into the U-tube shaped chamber 12 up to a level immediately below the conduits 18 and 22 and allowed to settle. After 24 hours, one liter of a saturated cuprous chloride chemically complexed solution 34 is placed in reservoir 10. The saturated solution 34 is complexed by saturating a 5 N hydrochloric acid solution with cuprous chloride. One liter of distilled water 36 is placed in reservoir 14. The solutions 34 and 36 are covered with a layer of paraffin oil, not shown, to reduce oxidation. After two weeks, crystals 38 begin to form in the gel 24 within the crystal growing chamber 12 as more clearly shown by referring to FIG. 5. Within one month, the crystals were still clear and were 6 mm. or larger. The largest clear crystals are 6 mm. on an edge while the largest clear crystals that could be produced by a conventional gel growth method were 3 mm. This represents an eight-fold increase in crystal volume.

Two factors that limit the ultimate crystal size in the usual gel growth methods are the depletion of the reactants and the increase in by-product concentration as the crystal grows. The apparatus of this invention reduces both of these factors. The volume of the reservoir 10 containing cuprous chloride is so large that the cuprous chloride concentration is not significantly decreased by removal of the cuprous chloride into the silica gel 24. The volume of the water reservoir 14 is so large that the hydrochloric acid liberated when the cuprous chloride crystals 38 are formed does not significantly increase the acidity of the water reservoir. Thus, in this apparatus, the concentration of hydrochloric acid and cuprous chloride along the length of the gel approaches a steady state condition because of the essentially constant concentrations at the gel interfaces. When this steady state is nearly reached, there will exist sites along the length of the gel where conditions are favorable for crystal growth and will remain favorable for a relatively long period of time. This steady state is not attained when crystals are grown by conventional techniques. If one tries to grow large crystals of cuprous chloride in a test-tube, the advancing acid front tends to dissolve crystals that have already been formed.

FIG. 2 represents a different embodiment of the apparatus of this invention showing the two reservoirs 10 and 14 interconnected respectively to chamber 12 by means of single conduits 26 and 28. The single conduits of FIG. 2 are of a larger diameter than the conduits of FIG. 1

and are employed to add structural stability to the apparatus. The double conduits 16, 18, 20 and 22 of FIG. 1 are utilized for mechanical stability and structural strength and either the double or single connecting conduits of FIGS. 1 and 2 are suitable.

5 FIG. 3 represents a further embodiment in which the crystal growing chamber 12 lies in a horizontal, centrally disposed relationship rather than the U-shaped form of FIGS. 1, 2 and 5. All the embodiments represented by FIGS. 1, 2, 3 and 5 are vented to the atmosphere and require the addition of a paraffin oil to the surface of the reactant solutions to prevent oxidation. FIG. 4, however, illustrates a closed system in which the reservoirs 10 and 14 are connected by means of clamps 30 and 32. In this embodiment, the utilization of a paraffin oil is not needed to prevent oxidation.

10 The apparatus of this invention has proved to be most effective in producing large single electromagnetic crystals in a simple and economical manner. Large crystals of cuprous chloride have been produced by the apparatus of 20 this invention and find particular use as modules for lasers.

15 While the invention has been described with particularity in reference to specific embodiments thereof, it is 25 to be clearly understood that the disclosure of the present invention is for the purpose of illustration only and is not intended to limit the invention in any way, the scope of which is defined by the appended claims.

#### What is claimed is:

30 1. An apparatus for growing single crystals within a gel matrix comprising, a first reservoir having a predetermined volume for the storage of a reactant material, a second reservoir having a predetermined volume for the storage of a reactant material, said first and second reservoirs being laterally spaced and disposed in a horizontal relationship, a crystal growing chamber of a size to allow for crystal growth positioned between said first and second reservoirs and operatively connected thereto to permit the establishment of a stationary, uniform reactant 35 concentration gradient within said growing chamber, said growing chamber having a predetermined volume for the storage of a gel matrix in which the ratio of the predetermined volume of the growing chamber to each of the predetermined volumes of the first and second reservoirs 40 is less than 1 to 10 and a gel matrix stored within said chamber.

45 2. An apparatus in accordance with claim 1 in which each of the first and second reservoirs are sealed from the atmosphere to prevent evaporation and oxidation of 50 the reactant materials.

55 3. An apparatus in accordance with claim 1 in which the crystal growing chamber forms a U-shaped tube and the gel matrix is disposed within the lower portion of the U-shaped tube and positioned below the horizontal level of the said operative connection.

#### References Cited

##### UNITED STATES PATENTS

|    |           |         |                    |        |        |
|----|-----------|---------|--------------------|--------|--------|
| 60 | 1,850,499 | 3/1932  | Francis            | -----  | 23—292 |
|    | 2,014,823 | 9/1935  | Tramm              | -----  | 23—292 |
|    | 2,532,257 | 11/1950 | Kirshenbaum et al. | 23—292 |        |
|    | 3,371,036 | 2/1968  | Torgesen et al.    | -----  | 23—301 |

##### OTHER REFERENCES

65 Modern Lab. Appliances, Fisher Scientific Co., p. 392 (1952).

Central Scientific Co. Catalog #H351 (1935), p. 571.

NORMAN YUDKOFF, Primary Examiner

70 R. T. FOSTER, Assistant Examiner

U.S. CL. X.R.

23—295, 300